

## UNITED STATES PATENT OFFICE

1,988,684

## PROCESS OF TANNING HIDES

Harold M. Gusdorf, Indianapolis, Ind.

No Drawing. Application November 17, 1932,  
Serial No. 643,053. Renewed April 12, 1934

7 Claims. (Cl. 149—4)

This invention relates to the art of tanning leathers and particularly to a method decreasing the length of time required heretofore in the tanning operation. Heretofore, the customary method has been to prepare the raw hides by removing the foreign matter such as hair, dirt, grease, loose flesh and the like, all in the usual manner well known to those versed in the art. The hides were then immersed in tanning liquors beginning first with a very weak liquor in respect to the tanning agent and then gradually increasing the strength of the liquor. Sufficient time had to elapse to permit the weaker liquor to thoroughly penetrate the hide before the next stronger liquor could be employed. If this process was speeded up to shorten the intervals of time between the applications of the succeeding, increasing strengths, the hides were damaged so that first class leather could not be produced. In employing this usual process of subjecting the hides to increasing strengths of liquor, the time required was generally in the neighborhood of from seven to twenty-five days. Were the hide to be placed at once in the strongest liquor, it would become damaged to such an extent as to become practically unusable.

This process heretofore employed is one requiring considerable attention and must be watched closely to insure that the fibers of the hide do not become damaged by too rapid subjection to the stronger liquors. It is essential in any process that the tanning materials be uniformly and thoroughly distributed through the hide to around the fibers therein.

By my invention I have been able to increase the speed with which the tanning materials will penetrate and completely tan a hide without damage thereto. My method consists essentially of using a liquid material non-injurious to the hide fibers which has a quick and thorough penetrating action on the raw prepared hide so as to have this material penetrate and fill all of the minute interstices within the hide and coat the surfaces of the fibers therein, giving the hide a solid and plump appearance, following which step the hide thus treated is submerged in a tanning liquor of the final strength to be employed, or at least of a strength much greater than that which has heretofore been possible to use on the raw hides. Within a relatively short time, the penetrating material initially employed will be found floating on the surface of the tanning material and the tanning material found to have penetrated uniformly

and completely through the hide, completely tanning the hide to give as good if not better leather than heretofore obtained in the longer, step by step, process of going from tanning materials of increasing strengths.

In other words, I employ what I believe to be purely a mechanical process wherein the fibers of the leather are first completely coated with films of protective material having less surface tension than a water tanning solution and a specific gravity less than water so that when the hide containing this material is submerged in a water solution of the tanning material this protective material will tend to gradually leave the hide by reason of the differences in specific gravity and permit the gradual replacement therewith of the tanning material. In short, my invention contemplates taking the hide which has been previously prepared for tanning, giving it a treatment with a protective material first holding out all of the tanning materials and then gradually replacing the protective material by the tanning materials as determined by the rate at which the protective material leaves the hide. This rate is determined by the differences in surface tension and specific gravity of the protective material and the tanning material solution.

The invention will be better understood by describing one particular way in carrying out the process. I take the hides after they have been initially prepared for tanning in the usual manner but instead of then subjecting the hides to tanning materials, I drop them in a vat containing the protective material to be employed. One particular protective material which I find to work very successfully is solvent naphtha in the crude form as distilled from coal tar having the approximate constants .862 to .892 specific gravity, 160 degrees C. boiling point (80 per cent) and a flash point of about 25.6 degrees C. The refined form may be used without noticeable difference in the results. An essential quality of the protective material is that it be a liquid capable of readily forming films about the hide fibers and have a surface tension slightly less than that of water films. The hide will be very shortly completely penetrated by the material employed, with the air and water driven out from between the fibers and adhering films of the material formed therearound as well as filling the interstices between the fibers. After the hides have been thoroughly penetrated by this material, the hides thus treated are removed from this protective material bath and

submerged in a vat containing the tanning material. This tanning material is in the form of a solution of the customary wood and bark in water but has a strength equal to that ordinarily employed as the strength in the last step of the process heretofore employed, the permissible strength being as high as 80 degrees, barkometer. The hides are left in this tanning vat until the tanning material has completely penetrated the 10 hides and displaced the protective material itself. This period of time will vary depending upon the thickness of the hides.

When the hides are placed in the protective material, they are submerged therein and a rapid ebullition of air is at once observed, indicating that the protective material is passing to within in the hides to displace the air which has been entrapped therein. When the hides treated with this material are placed in the tanning solution, 20 the hides are submerged and an accumulation of the protective material is soon observed floating on the top of this solution. By reason of the fact that the hides are submerged and also of the fact that the difference in specific gravity 25 of this protective material and of the water tanning solution, the protective material will leave the hides, not too rapidly but gradually and continuously, and as it does so, the tanning solution will of course flow in to replace this material as it leaves. When the interchange of these materials is complete, the hides are thoroughly tanned and are taken from the vat to be subjected to further conditioning treatment as is the usual practice.

35 The protective material initially holds back the strong tanning solution so as to prevent burning of the fibers, and the tanning solution is only admitted to the fibers as the protective material leaves. The rate of interchange seems 40 to be ideal in that the fibers are uniformly subjected to a gradually increasing amount of the tanning solution at just the right speed to give a thorough tanning without drawing and burning the hides.

45 I believe that what actually occurs in practicing my invention is to be explained as follows. The hides as initially prepared for tanning are full of water and contain some air. When the hides are immersed in the liquid protective material which does not diffuse in water and has less surface tension than that of water, the water films about the hide fibers are rapidly replaced by the protective liquid films so as to completely enclose them. Then when the hides 50 thus protected are submerged in the bath of tanning liquor having water as the solvent, as between the surface tension of the protective material and of the liquor, the protective material tends to remain, but being submerged, its 55 buoyancy tends to break its adhesion to the fibers and, together with the increased pressure applied to what air may be within the fibers, the protective material thus leaves the fibers not violently but gradually since the net operating 60 forces are relatively small. The films of protective material become thinner and thinner until they puncture and permit the tanning liquor to break through in small quantities first, and then in increasingly larger quantities until the replacement is complete, the protective films all the time still fighting against gravity to displace 65 the water films.

70 There is the further possible action, in that the protective liquid initially displaces air from 75 the voids between fibers in the hides, so that

when the protected hides are submerged in the water tanning solution, the surface tensions then to be considered are those of the protective liquid, the tanning liquid and the solid fibers. By eliminating the air, then the surface tensions between the air and liquid and between the air and water are eliminated, leaving but the surface tension between the liquid and the water. The situation arises where two liquids are in contact in the absence of air but adjacent solid fibers, in which case, the liquids will move in the direction in which the surface-pressure at the solid is least, and since the protective liquid is adjacent the fiber when the tanning liquor is applied, then the tanning liquor would drive or "chase" the protective fluid along and off the fibers to allow the tanning liquors to come into contact gradually with the fibers.

In following the above process in accordance with my invention, the raw hide is completely 20 tanned within a much shorter period than permissible with the method heretofore employed. In comparison, I have found in tanning like hides, that, for a hide of approximately 1/12 of an inch thickness, the old method has required 25 from five to six days to completely tan the fibers, whereas by my invention, the same result is obtained in from 12 to 24 hours. This decrease in time required for tanning is not secured at the expense of a lower quality of leather but instead 30 I find that the leather tanned by this new process to be of the same if not better quality than that obtained by the old process.

While I have herein described one particular way in practicing my process, it is to be understood that my invention resides in the subjecting of the hides to the penetrating material followed by a second step of subjecting the hides thus treated to a relatively strong tanning solution to secure a replacement of the penetrating 40 material by the tanning material, and that the invention is not limited to the particular handling herein set out.

I claim:

1. In the process of tanning hides, the combination of those steps which comprise the step of preparing the hides for tanning, the step of immersing the prepared hides in a liquid protective material having a specific gravity differing from that of a water solution of tanning material to be employed to secure a thorough penetration of the material through the hides, and the step of then immersing the hides in a bath of relatively strong water solution of tanning material and retaining the hides in the bath until the tanning solution has displaced the protective material.

2. The method of tanning hides which includes initially preparing the hides for tanning, immersing and retaining the prepared hides in a solvent naphtha bath until the hides are thoroughly penetrated thereby, and then immersing and retaining the hides in a bath of a water solution of tanning materials until the solvent naphtha is replaced by the tanning material.

3. The method of tanning hides, which includes initially preparing the hides for tanning, soaking the hides in a protective material lighter than the solution of tanning material to be employed until the material has thoroughly penetrated the hides, and then flowing out that protective material in water in the presence of a relatively strong concentration of tanning materials.

4. The method of tanning hides which comprises initially preparing the hides for tanning, coating the fibers in the hides with films of a protective liquid having a surface tension slightly less than that of water, and then replacing those films with films of a water solution of tanning materials, and applying pressure to the hides to accelerate the rate of replacement of said liquid films by the water films.
- 10 5. The method of tanning hides which comprises initially preparing the hides to leave films of water about the fibers in the hide in the presence of air, subjecting the water films in the presence of the air to films of a protective liquid having a surface tension between it and the water film less than the sum of the surface tensions between the air and the water, and the air and the liquid whereby the water films are replaced by protective liquid films, filling the voids between the fibers in the hides with the protective liquid to expel the air, floating out the protective liquid from the voids in the hides in the absence of air and in the presence of a water tanning solution wherein the surface tension of the tanning solution is less than that of the surface tension of the protective liquid,

and continuing the application of the tanning solution to the hides to cause a displacement of the protective liquid films by films of the tanning solution.

6. In the process of tanning hides, the combination of those steps which consist of the step of treating the hides with a liquid, water insoluble, protective penetrating material having a specific gravity less than that of the tanning solution to be employed to fill the voids and coat the fibers in the hides, and the following step of interchanging that protective material with the tanning solution by relative flows of the material and the solution induced by differences in specific gravities and surface tensions therebetween.

7. In a method of treating a hide wherein the hide is subjected to a tanning liquor, those steps which include the step of immersing the hide immediately preceding the application of the tanning liquor thereto in an oil having more surface tension than that of the liquor, and the succeeding step of immersing the oil plumped hide in the liquor to permit an interchange of the liquor with the oil.

HAROLD M. GUSDORF.

**CERTIFICATE OF CORRECTION.**

**Patent No. 1,988,684**

**January 22, 1935.**

**HAROLD M. GUSDORF.**

**It is hereby certified that error appears in the printed specification of the above numbered patent requiring correction as follows: Page 1, second column, line 10, for "a water tanning solution" read water; and line 11, for "water" read a water tanning solution; and that the said Letters Patent should be read with these corrections therein that the same may conform to the record of the case in the Patent Office.**

**Signed and sealed this 28th day of May, A. D. 1935.**

**Leslie Frazer**

**(Seal)**

**Acting Commissioner of Patents.**